

# United States Patent Office.

CYRUS MOORE, OF EAST SAGINAW, ASSIGNOR TO HIMSELF AND ABEL BLAKESLEE, OF DETROIT, MICHIGAN.

*Letters Patent No. 70,454, dated November 5, 1867.*

## IMPROVED LUBRICATING OIL.

*The Schedule referred to in these Letters Patent and making part of the same.*

TO WHOM IT MAY CONCERN:

Be it known that I, CYRUS MOORE, of East Saginaw, in the county of Saginaw, and State of Michigan, have invented a new and useful Method of Manufacturing Lubricating Oil; and I do declare that the following is a just and accurate description thereof.

I will describe the manufacture of a given quantity of ten gallons of the oil, and give the proportions of each of the ingredients used, so that any one can make their own calculations of the quantities of each necessary to be used in the manufacture of any other given quantity.

Take ten gallons of coal tar, brought to a boiling heat, and then run it through any proper rectifier, to separate any earthy or other impure matter from it. After rectifying the coal tar, add to it one gallon of benzine, one gallon of sperm oil, and one quart of alcohol. The result will produce a fine lubricating oil.

What I claim as my invention, and desire to secure by Letters Patent, is—

1. The method of manufacturing a lubricating oil by the process described.
2. The use of the ingredients, and in the proportions substantially as described, for the purpose designed.

CYRUS MOORE.

Witnesses:

H. F. HANNAMAN,  
A. M. SPRAGUE.